

# UNITED STATES PATENT OFFICE.

FREDERICK G. KEYES, OF CAMBRIDGE, MASSACHUSETTS, ASSIGNOR TO COOPER HEWITT ELECTRIC COMPANY, A CORPORATION OF NEW JERSEY.

## MANUFACTURE OF MOLYBDENUM-TUNGSTEN ALLOY.

1,377,982.

Specification of Letters Patent. Patented May 10, 1921.

No Drawing. Original application filed October 16, 1915, Serial No. 56,214. Divided and this application filed July 11, 1917. Serial No. 179,933.

To all whom it may concern:

Be it known that I, FREDERICK G. KEYES, a citizen of the United States, and resident of Cambridge, county of Middlesex, State of Massachusetts, have invented certain new and useful Improvements in the Manufacture of Molybdenum-Tungsten Alloy, of which the following is a specification.

The present invention relates to a new method of producing an alloy of tungsten and molybdenum containing any desired percentage of the last named element. Such an alloy may be used for a great variety of purposes and it is not my intention to describe it in such a way as to confine its use necessarily to any particular art. In order, however, to point out one important use of this alloy, I shall with the reservation above made, describe it as suited to the purposes of making lamp filaments or resistance wire for electric tube furnaces. For this purpose I have found that an alloy of pure tungsten with twenty per cent. of molybdenum, for example, is highly satisfactory. For other purposes and possibly also for the purpose of making a wire such as last described, other proportions of molybdenum and tungsten may be found usable. I may say that it appears to be only necessary that there should be enough of the molybdenum present, so that when the same is liquefied by a heating process, there shall be enough liquid present to pull together the particles of powdered tungsten which, as will appear, are mixed with the molybdenum oxide particles at the beginning of the process. The description herein will be concerned more particularly with the manufacture of an alloy of eighty per cent. tungsten and twenty per cent. of molybdenum, although it is not intended to exclude other proportions of molybdenum in combination with tungsten, if manufactured in accordance with the process about to be described.

It is known that molybdenum has a melting point lying approximately 500° C. below the melting point of tungsten. Now, when a bi-metallic mixture of fine particles of molybdenum and tungsten is gradually heated by any suitable means, preferably by passing an electric current through it, the lower melting constituent will melt first, and if it be present in sufficient quantity will, owing to its surface tension, tend to

draw the mass of powdered material together into a coherent ingot. The following process is suited for producing conveniently an alloy of molybdenum and tungsten. By taking quantities of chemically pure  $\text{MoO}_3$  and  $\text{WO}_3$  and reducing the mixture to a metallic state, an alloy of the desired metallic Mo content will result. This content may be twenty per cent. molybdenum or any other percentage which is found preferable.

It is better to mix the oxids previously to reducing to the metallic state rather than to attempt to mix the metals after reduction, owing to the fact that a much more uniform mechanical mixture can be produced in this way, on account of their being soft and capable of being reduced by means of a pestle or other grinding agent.

It will be understood that the oxids are first thoroughly ground and mixed. Thereafter they are reduced either by means of dry  $\text{CO}$  or dry  $\text{H}_2$ . When reducing with  $\text{H}_2$ , the reduction should be carried slowly to completion at about 800° and finished at about 1000°. The coarseness of the mixture reduced by hydrogen depends on the speed of the gas stream. A very slow gas stream will require a longer time for the reduction and yield a coarser powder than a reduction carried out at the same temperature with a rapid stream of dry hydrogen. It would seem that the pressure of the water vapor which is not promptly carried off, as it would be with a vigorous stream of hydrogen, causes a growth of small particles to larger particles by some alternate reduction and oxidation action. For the purpose specially desired to be served by the present invention it is desirable to have fine and thoroughly reduced metal.

The metal, having been suitably reduced, is mixed with a little water and molded to a bar under pressure. During the drying of the molded bar the finer particles undoubtedly oxidize superficially. The dry bar is placed in a furnace maintained at about 1200° and through it a very slow stream of dry hydrogen is caused to pass. After about an hour heating, the bar may be allowed to cool in  $\text{H}_2$ . The bar of metal so produced is sufficiently strong to permit of its being handled. The cohering appears to be due to the slow reduction of the super-

ficially oxidized particles. The bar produced in the above manner when cooled, is further heated by the passage of the electric current until its temperature has attained 5 the melting point of molybdenum. At this temperature the molten molybdenum begins to alloy with the tungsten particles and, owing to the surface tension of the liquid molybdenum, the particles of tungsten are 10 pulled together. In carrying out this process it is essential to maintain the bar at the proper temperature until contraction ceases.

The bar thus produced may be rolled into 15 sheets at 800 to 900° C. The material is quite soft while hot and may be drawn into wire by the ordinary drawing process applied to most metals.

I prefer for many purposes, as has been 20 stated, to make the proportions of molybdenum and tungsten respectively twenty per cent. and eighty per cent.

An alloy produced in the manner described and drawn into wire is admirably suited to serve the purposes of a filament for 25 electric lamps and of resistance for electric furnaces and like purposes.

This application is a division of my application Serial Number 56,214, filed October 16th, 1915.

30 I claim as my invention:

1. The step in the method of producing a bar of metallic alloy composed of molybdenum and tungsten which consists in subjecting a molded moistened bar of said

metals to a drying process, applying to the 35 dry bar a heat of about 1200° and passing through it a very slow stream of dry hydrogen.

2. The step in the method of producing a bar of metallic alloy composed of molybdenum and tungsten which consists in subjecting a 40 molded moistened bar of said metals to a drying process, applying to the dry bar a heat of about 1200° and passing through it a very slow stream of dry hydrogen for about an hour, and cooling the bar in H<sub>2</sub>.

3. The method of producing a bar of metallic alloy composed of molybdenum and tungsten which consists in subjecting a 45 molded bar of said metals to a drying process, applying to the dry bar a heat of about 1200° and passing through it a very slow stream of dry hydrogen for about an hour, and cooling the bar in H<sub>2</sub>, afterward further heating the bar by passing an electric current therethrough until it has attained the melting point of molybdenum and maintaining the bar at approximately the temperature named until contraction ceases. 50

Signed at Cambridge in the county of Middlesex and State of Massachusetts this 9th day of July A. D. 1917.

FREDERICK G. KEYES.

Witnesses:

WALTER HUMPHREYS,  
WILLIAM JACKSON.